



US008814953B1

(12) **United States Patent**  
**Abbott et al.**

(10) **Patent No.:** **US 8,814,953 B1**  
(45) **Date of Patent:** **Aug. 26, 2014**

(54) **SYSTEM AND METHOD FOR SPRAY DYEING FABRICS**

(75) Inventors: **Michael D. Abbott**, Statesville, NC (US); **Robert A. Miller, III**, New Ringgold, PA (US); **Ruth E. May**, Schuylkill Haven, PA (US)

(73) Assignee: **HBI Branded Apparel Enterprises, LLC**, Winston-Salem, NC (US)

(\*) Notice: Subject to any disclaimer, the term of this patent is extended or adjusted under 35 U.S.C. 154(b) by 75 days.

(21) Appl. No.: **12/371,812**

(22) Filed: **Feb. 16, 2009**

|               |         |                      |
|---------------|---------|----------------------|
| 2,985,502 A   | 5/1961  | Kronsbein et al      |
| 2,990,087 A   | 6/1961  | Brewin et al         |
| 2,990,088 A   | 6/1961  | Isken et al.         |
| 3,022,926 A   | 2/1962  | Bailey, Jr.          |
| 3,181,749 A   | 5/1965  | Storr et al          |
| 3,978,557 A * | 9/1976  | Goodson .....        |
| 4,612,016 A   | 9/1986  | Jaeger et al.        |
| 4,659,333 A   | 4/1987  | Schaub               |
| 4,717,391 A   | 1/1988  | Daniel et al.        |
| 4,786,721 A   | 11/1988 | Tzikas et al.        |
| 5,010,612 A   | 4/1991  | Jensen et al.        |
| 5,016,308 A * | 5/1991  | McBride et al. ....  |
| 5,205,305 A   | 4/1993  | Yamakita             |
| 5,288,322 A   | 2/1994  | Hanna et al.         |
| 5,458,265 A   | 10/1995 | Hester et al.        |
| 5,593,072 A   | 1/1997  | Hester et al.        |
| 5,713,223 A * | 2/1998  | Lin .....            |
| 5,951,717 A * | 9/1999  | Mrotzcek et al. .... |
| 5,964,407 A   | 10/1999 | Sandkleiva           |
| 6,063,137 A   | 5/2000  | Scheibl et al.       |

(Continued)

**Related U.S. Application Data**

(63) Continuation-in-part of application No. 11/395,848, filed on Mar. 31, 2006, now Pat. No. 7,799,097, which is a continuation-in-part of application No. 10/601,820, filed on Jun. 23, 2003, now Pat. No. 7,033,403.

(51) **Int. Cl.**  
**D06P 7/00** (2006.01)

(52) **U.S. Cl.**  
USPC ..... **8/499**; 28/169

(58) **Field of Classification Search**  
USPC ..... 8/149.1  
See application file for complete search history.

(56) **References Cited**

**U.S. PATENT DOCUMENTS**

|               |         |              |
|---------------|---------|--------------|
| 1,893,197 A * | 1/1933  | Cohn .....   |
| 2,915,230 A   | 12/1959 | Brewin et al |
| 2,974,838 A   | 3/1961  | Parham       |

**FOREIGN PATENT DOCUMENTS**

|    |          |        |
|----|----------|--------|
| DE | 19633101 | 2/1998 |
| EP | 1233098  | 8/2002 |

(Continued)

*Primary Examiner* — Harold Y. Pyon

*Assistant Examiner* — Katie L Hammer

(74) *Attorney, Agent, or Firm* — Womble Carlyle Sandridge & Rice LLP

**ABSTRACT**

A system and method are provided for dyeing fabric, the system including a dye spray station, a dye fixation station downstream of the dye spray station, and at least one rinse station downstream of the dye fixation station. The process includes opening the fabric with a spreader to maintain the fabric flat and taut, spraying the outer surfaces of the fabric with a dye, and exposing the fabric to atmospheric steam to chemically react and affix the dye to the fabric.

**19 Claims, 4 Drawing Sheets**



(56)

**References Cited**

U.S. PATENT DOCUMENTS

|                 |         |                 |       |        |
|-----------------|---------|-----------------|-------|--------|
| 6,120,560 A *   | 9/2000  | Miller et al.   | ..... | 8/483  |
| 6,393,871 B1 *  | 5/2002  | Chiang          | ..... | 68/5 D |
| 6,443,569 B1    | 9/2002  | Mheidle et al.  |       |        |
| 6,471,729 B1    | 10/2002 | Voth et al.     |       |        |
| 7,144,431 B2    | 12/2006 | Gardner et al.  |       |        |
| 2002/0138922 A1 | 10/2002 | Schmiedl et al. |       |        |

|                   |        |             |       |           |
|-------------------|--------|-------------|-------|-----------|
| 2003/0033950 A1 * | 2/2003 | Matich      | ..... | 101/424.2 |
| 2004/0154146 A1 * | 8/2004 | Pruitt, Jr. | ..... | 26/99     |

FOREIGN PATENT DOCUMENTS

|    |               |        |
|----|---------------|--------|
| EP | 1275700       | 1/2003 |
| IT | PD2001A000089 | 4/2001 |
| WO | 9628604       | 9/1996 |

\* cited by examiner



FIG. 1



FIG. 2



FIG. 3



FIG. 4



FIG. 5

## SYSTEM AND METHOD FOR SPRAY DYEING FABRICS

### RELATED APPLICATIONS

This application is a continuation-in-part of U.S. application Ser. No. 11/395,848, filed Mar. 31, 2006 now U.S. Pat. No. 7,799,097, which is a continuation-in-part of U.S. application Ser. No. 10/601,820, filed Jun. 23, 2003 now U.S. Pat. No. 7,033,403, the contents of which are incorporated by reference herein.

### FIELD OF THE INVENTION

The present invention is related to fabric coloring. More particularly, the present invention is related to a system and method for spray dyeing and/or bleaching fabrics.

### BACKGROUND OF THE INVENTION

Today, fabrics are made from a wide variety of natural fibers, such as cotton, synthetic fibers, and combinations thereof. The basic fabric is a greige fabric that must be dyed and/or bleached in order to provide the desired color to the resultant fabric and/or garment. Many dye compositions and methods have been proposed for dyeing fabrics; however, dyeing greige fabric remains costly in terms of materials, labor, and/or processing time.

One conventional dyeing method, known as yarn dyeing, involves dyeing individual fibers or yarns prior to the fibers or yarns being sewn, knitted, or woven into a fabric. A significant problem associated with this method is the substantial inventory requirement to maintain a supply of the various colored yarns needed to produce various products, and the prohibitively high inventory costs resulting therefrom.

Another conventional dyeing method is known as bulk dyeing. In bulk dyeing, un-dyed fibers or yarns are knitted or woven into a raw or undyed fabric. The raw fabric is subsequently scoured or bleached, and then dyed.

Common bulk dyeing methods include vat dyeing, beam dyeing, jet dyeing, and bath dyeing. Vat dyeing typically consists of immersing a piece of fabric in a vat of liquid dye. Beam dyeing involves winding a length of fabric about a perforated beam. The beam is then placed in a vessel where dye is pumped into the center of the beam, out of the perforations, and through the fabric. Jet dyeing involves placing the fabric in a high-pressure, high-temperature kettle of liquid dye. Bath dyeing involves immersing the fabric in a bath of dye in a rotating drum.

There are a number of problems, however, associated with bulk dyeing methods. First, the bulk dyeing process necessitates large volumes of water, which increases the costs of the bulk dyed fabrics, and has an adverse impact on the environment and conservation of natural resources. Also, some of the dyed fabric must be cut away from templates during the manufacture of a garment from the fabric. Since the bulk fabric has already been dyed, this results in increased costs due to the wasted dye and fabric.

A more significant problem with bulk dyed fabrics in the manufacture of garments is the unpredictability of consumer color preferences. In the garment industry, changes in consumers' preferences for one color over another color can lead to an overstock of the undesired colored garments and a back-order of the desired colored garments.

Other methods of dyeing fabrics involve printing dyes onto a surface of a fabric. These methods are commonly used to apply a decorative pattern on the surface of the fabric. Such

printing methods include screen-printing and inkjet printing. While these methods have proven useful in quickly changing from one decorative pattern to another, they have not proven useful for large scale production of fabrics or garments.

Accordingly, there is a continuing need for flexible, low cost, low waste processes for dyeing fabrics.

### BRIEF DESCRIPTION OF THE DRAWINGS

10 FIG. 1 is a schematic view of an exemplary embodiment of the system for dyeing and/or bleaching fabric according to the present invention.

FIG. 2 is a perspective view of the ring guides and the scroll roll of the exemplary embodiment of the system of FIG. 1.

15 FIG. 3 is a schematic view of the spray dyeing station of the present invention.

FIG. 4 is a schematic view of the rinsing stations of the present invention.

20 FIG. 5 is a schematic view of the collection unit of the present invention.

### DETAILED DESCRIPTION OF THE INVENTION

Referring to the figures in general, and to FIG. 1, in particular, one aspect of the present invention is directed to a system, shown generally as reference numeral 100, for continuously dyeing a fabric. Another aspect of the present invention, as described herein, is the method for continuously dyeing a fabric with reference to the system.

30 In one exemplary embodiment, the system 100 comprises a fabric positioning station 110, a spray station 120, a fixation station 150, and at least one rinse station 160. As described in greater detail below, the system 100 may further comprise a drying unit 180 or a fabric handling station 190 (shown in FIG. 4). Shown generally as reference numeral 14, the fabric 14 may be a tubular knit fabric in its un-dyed or raw (greige) state, although the invention is not limited to dyeing tubular knit fabric. Indeed, any fabric substrate can be dyed using the system and method of the present invention.

40 In one exemplary embodiment, fabric 14 is drawn from a supply of fabric, such as a knitting machine or fabric roll 12 by a downstream roller 117, as described in greater detail below. As shown in FIG. 1, at the fabric positioning station 110, folds are removed from the fabric 14. For example, the fabric 14 may be drawn through opposed ring guides 112, on either side of the flat fabric 14, over a spreader bar 114, or former, that opens the tubular fabric 14. As shown in FIG. 2, the ring guides each comprise a pair of balls, which rotate about a vertical axis to engage and hold the fabric 14 taut. The spreader 114 ensures that the fabric is flat and, thus, any folds or creases in the fabric are substantially removed.

45 After passing over the spreader 114 and through the ring guides 112, the fabric is allowed to relax as it passes beneath roller 115, which serves to maintain the appropriate tension on the fabric and guide the fabric to a driven scroll roll 117. As best shown in FIG. 2, the scroll roll 117 is a roller having a rubber outer coating with angled, raised ribs 117a, which diverge outwardly from the center of the roller toward the opposed ends 117b of the scroll roll 117. As the scroll roll 117 rotates, drawing the fabric 14 across the top of the roller 117, the ribs pull the fabric outwardly to keep it taught and smooth.

50 The fabric 14 is next drawn through the spray station 120 by downstream rollers 154, where at least one surface, i.e., the technical face or technical back, of the fabric is sprayed with dye. As illustrated schematically in FIG. 1, in one embodiment the spray station 120 comprises upper and lower portions 120a and 120b, for spraying both technical faces of the

55

flat tubular fabric 14. Referring to FIG. 3, the spray station 120 is shown in greater detail. A vessel 121 holds the desired volume of a dye composition, such as a reactive dye mixture. The terms "reactive" or "reacts," as used herein, refer to the reaction of the dye with the fabric that results in the formation of an attachment to one or more components of the fabric, such as by a covalent bond. Suitable reactive dye compositions are described in U.S. Pat. No. 4,786,721 and in pending U.S. patent application Ser. Nos. 11/338,346, 11/656,769, and 12/329,684, which are incorporated herein by reference. The present invention reduces the amount of water required for dyeing the fabric. Specifically, whereas conventional dyeing processes require about a 6:1 ratio of water to dye, the system and method of the present invention require only about a 1:6 ratio of water to dye.

The dye composition is drawn from the vessel 121 by fluid pumps 122. As shown in FIG. 3, where the spray station comprises upper and lower portions 120a and 120b, the system 100 comprises two parallel paths and two fluid pumps 122a, 122b in parallel. To regulate the volume of dye composition sprayed onto the faces of the fabric 14, the dye composition is pumped through flow meters 123a, 123b, which are selectively set for the particular fabric type and construction, as well as the type and composition of the dye composition. The dye composition next moves through pressure regulators 124a, 124b where the pressure of the spray also is selectively set, depending upon the width of the fabric and the percentage of wet pickup needed for penetration of the dye. In one exemplary operation, the pressure of the spray is about 40 pounds per square inch. Lastly, the dye composition is delivered to manifolds 126a, 126b, each manifold 126 being in fluid communication with a plurality of spray nozzle heads 127a, 127b. In the embodiment shown in FIG. 3, each manifold 126 has three spray nozzle heads 127; however, the actual number of spray nozzle heads is dependent upon factors that include width of the fabric being sprayed.

The spray nozzle heads 127 apply the dye composition to the top and bottom surfaces, i.e., technical faces, of the open fabric 14 with dye. In one exemplary embodiment, the spray nozzles are arranged to deliver the dye composition to cover an angle of 110 degrees or less, as measured from the center of the manifolds 126a, 126b. As will be appreciated, this coverage is dependent upon the width of the fabric and the distance between the spray nozzles 127 and the face of the fabric 14. More particularly, the spray nozzles are arranged so that the dye is applied up to, but not beyond, the edges of the fabric, such that there is no overspraying of the fabric and no wastage of dye. This permits the dye to migrate around the edges of the fabric and through the fabric. Additionally, the spray nozzles are configured so that the dye composition is sprayed evenly across the width of the fabric. Further, the spray nozzles are sized, and the settings of the flow meters 123 and pressure regulators 124 selected to achieve between about 65 percent and 85 percent saturation of the total fabric, i.e., the percentage of the maximum amount that the fabric can hold.

The fabric positioning station 110 and the spray station 120 described herein are equally effective in applying a bleach composition to the fabric 14. For bleaching applications, the system may be configured so that the bleach composition and optical brighteners are mixed at the spray nozzles 127 via a separate fluid line (not shown). A suitable bleach composition is described in pending U.S. patent application Ser. No. 12/329,680, also incorporated herein by reference. The particular fabric construction and the constituents of the bleach composition will determine the extent to which the remaining portions of the system 100 described herein may be employed

to treat the bleached fabric; however, it is contemplated that the system may be used to further treat the bleached fabric, such as applying softeners, stain releases, wicking agents, etc.

In some embodiments of the present invention, the system 5 further comprises one or more heating devices 130 positioned between the spray station 120 and the downstream fixation station 150. The heating devices are set to initiate the chemical reaction of the dye.

The dyed fabric 14 is next drawn over a guide roller 129 and 10 through the fixation station 150 by rollers 154a, where the dyed fabric 14 is exposed to atmospheric steam, i.e., steam at atmospheric pressure, before the dye dries on the fabric. As discussed above, the color fixation station 150 exposes the fabric 14 to steam and heat in a manner and amount sufficient 15 to spread the dye throughout the fabric, i.e., from the technical face to the technical back, and affix the dye to the fabric as the fabric is continuously moved through the station 150. As shown in FIG. 1, the color fixation station 150 comprises a steam box 152, and a plurality of rollers 154a, 154b for 20 transporting the fabric through the steam box 152 in a lengthy path, exposing both technical faces of the fabric to similar conditions. In one embodiment, only the uppermost rollers 154a are driven. More particularly, steam entering the steam box maintains the exposure temperature in the steam box 152 at between about 196 degrees Fahrenheit and 210 degrees Fahrenheit, and at a relative humidity of between about 60 percent and 90 percent. In one embodiment, the arrangement and rotational speed of the rollers 164 creates a path through the steam box of about nine yards (27 feet) and a dwell time 25 within the steam box 152 of between about three minutes and four minutes. While FIG. 1 schematically shows five rollers 154a, 154b, the number of rollers may be increased or decreased depending upon the desired amount of exposure of the fabric 14 to the steam.

35 Of course, it is contemplated by the present disclosure for rollers 154 to be horizontally arranged, angled with respect to the horizontal or vertical, or combinations thereof. It is also contemplated to adjust the speed of rollers 154 with respect to one another so that the fabric 14 relaxes as it moves through 40 the fixation station 150. Advantageously, the rollers 154 are configured to minimize surface contact with the fabric 14 during the fixation process.

Following fixation of the dye in the fixation station 150, the dyed fabric is advanced through ring guides 153 into at least 45 one rinse station. Again, the ring guides 153 hold the fabric taut as it advances into the first rinse station. As shown in FIG. 1, in one embodiment there are two stations provided, shown as 160 and 170, respectively. The fabric also may be overfed into the first rinse station 160 to reduce residual stresses in the fabric.

50 Turning to FIG. 4, the rinse stations 160 and 170 are shown in greater detail. Upon passing into the first rinse station 160, the fabric 14 is sprayed with pressurized hot water having a temperature of between about 100 degrees Fahrenheit and 55 180 degrees Fahrenheit, with about 160 degrees Fahrenheit being preferred. The use of pressurized hot water ensures the minimal use of water in the rinse process. Upon entering the first rinse station 160, the fabric is drawn through ring guides 163 by downstream nip rollers 167 before spray nozzles 161 and 163 direct a pressurized spray vertically upward and 60 vertically downward against the fabric. The spray action of these nozzles serves two functions. First, the vertical action of the pressurized spray cleans the dyed fabric, removing any unaffixed hydrolyzed dye, residual chemicals, and insolubles 65 from the fabric 14. Second, the pressurized action of the vertically directed nozzles serves to compact the tubular knitted fabric 14. As the fabric approaches a first set of nip rollers

167, two additional spray nozzles 165 are directed angularly upward and angularly downward toward the entrance to the nip rollers 167 to further clean and to further compact the tubular knitted fabric by the mechanical action of pushing the knitted loops (courses) of the fabric 14 against the nip rollers 167. This effectively reduces the subsequent residual shrinkage in the fabric and apparel formed therefrom.

Each of the nozzles 161 and 165 deliver about 2.6 gallons of fluid per minute at a pressure of about 1,800 pounds per square inch, for a spray volume of about six gallons per linear yard of fabric 14. The cleaning fluid mixture comprises water at a temperature of about 160 degrees Fahrenheit, and a neutralizing agent. One suitable neutralizing agent is acetic acid. If the fabric is being bleached instead of being dyed, a peroxide scavenger is also added to the mixture. Upon passing through the first set of nip rollers 167, about 60 percent of the excess rinse water and chemical mixture is extracted from the fabric 14. In addition to substantially reducing the volume of water required for the cleaning and treatment at the first rinse station 160, the resulting extracted hydrolyzed dye and liquid are not environmentally harmful.

After passing through the nip rollers 167, the fabric is drawn through ring guides 173 by downstream nip rollers 177 where two spray nozzles 175, angled in the same fashion as the angled spray nozzles 165, further compact the fabric 14 as it enters the second set of nip rollers 177. The nozzles also may apply a finish such as a softener and water composition. Spray nozzles 175 also deliver about 2.6 gallons per minute at a pressure of about 1,200 pounds per square inch, for a total volume of about six gallons per linear yard. Upon passing through the nip rollers 177, approximately 60 percent of the excess rinse water and softener finish is extracted.

In some embodiments, one or more of the rinse stations may provide a pH adjustment. Alternatively, the system 100 may comprise a third rinse station 180, shown in FIG. 4, wherein the rinse water has a predetermined pH level so that the rinse water adjusts the pH of the dyed fabric to a pH that is neutral or slightly acidic. Any of the rinse stations may further deliver a fragrance, a stain repellent component, a water repellent component, etc. Additionally, the first set of nip rollers 167 and second set of nip rollers 177 may have differential rotational speeds; i.e., the speed of the first set 167 may be greater than the speed of the second set 177, thus overfeeding to the second set 179 to further facilitate compaction. The pressure applied by the nip rollers 167, 177 sets the moisture level remaining in the fabric 14 to between about 20 percent and 60 percent saturation.

In one embodiment, the system 100 of the present invention is configured to recirculate rinse water from the rinse stations to further reduce the amount of water consumed during the dyeing and finishing of the fabric 14. As will be appreciated by those in the art, the rinse water collected in the rinse station basis of the most downstream rinse station will be the cleanest, as it will contain the least hydrolyzed dye, chemicals, and/or insolubles. Thus, as shown by the arrows, W, collected rinse water from rinse station 180 is recirculated to the spray nozzles 175 in the second rinse station 170. Similarly, the collected rinse water from the second rinse station 170 is recirculated to the spray nozzles 165 in the first rinse station 160. Finally, the rinse water from the first rinse station 160 is drained or pumped for wastewater disposal.

Upon exiting the second rinse station 170, or third rinse station 180, if included in the system configuration, the system and process may comprise a collection unit 190 for the finished, wet fabric 14. An exemplary embodiment of a collection unit 190 according to the present disclosure is shown

in FIG. 5. The collection unit 190 includes an opening unit 191, an inclined relaxing conveyor 195 a platter 196 and a fabric receptacle 198.

As shown in FIG. 5, as the fabric 14 exits the second rinse station 180, it is opened by the opening unit 191. The fabric is engaged by a final set of edge drives 193, which set the width of the fabric for the subsequent collection and drying. The fabric 14 is then deposited onto the inclined relaxing conveyor 195 in a tensionless state. The fabric 14 exits the conveyor 195 via the platter 195 and is collected in the fabric receptacle 198.

While the present invention has been described with reference to one or more exemplary embodiments, it will be understood by those skilled in the art that various changes may be made and equivalents may be substituted for elements thereof without departing from the scope of the present invention. In addition, many modifications may be made to adapt a particular situation or material to the teachings of the disclosure without departing from the scope thereof. Therefore, it is intended that the present invention not be limited to the particular embodiment(s) disclosed as the best mode contemplated for carrying out this invention, but that this invention will include all embodiments falling within the scope of the present disclosure.

The invention claimed is:

1. A system for dyeing fabric, the fabric being tubular, comprising:

(a) a fabric positioning station comprising:

(i) a spreader bar or former that opens and substantially flattens the fabric with a first outer surface of the fabric above the spreader and a second outer surface of the fabric below the spreader, the fabric having a width;

(ii) a roller downstream of the spreader for drawing the flattened fabric from the spreader, the roller having a plurality of raised ribs for maintaining tension in the fabric;

(b) a dye spray station downstream of the fabric positioning station for receiving the fabric comprising:

(i) a first dye supply manifold and a second dye supply manifold;

at least one spray nozzle in liquid communication with each dye supply manifold for spray dyeing the flattened fabric evenly across the width of the first and second outer surfaces of the fabric, respectively;

(c) a dye fixation station downstream of the dye spray station for receiving the dyed fabric, wherein the dye is chemically affixed to the fabric; and

(d) at least a first rinse station downstream of the dye fixation station for receiving the dyed fabric, wherein residual materials are removed from the dyed fabric.

2. The system of claim 1 further comprising:

(a) a dye supply source;

(b) a fluid pump for transferring the dye from the dye supply source through a flow meter to regulate the flow of dye through the at least one spray nozzle; and

(c) a pressure regulator downstream of the flow meter to regulate the pressure of the dye to the dye supply manifold and through the spray nozzle.

3. The system of claim 1 wherein the dye fixation station comprises:

(a) a steam box for receiving spray dyed fabric from the dye spray station and exposing the spray dyed fabric to steam at atmospheric conditions; and

(b) a plurality of rollers arranged to move the spray dyed fabric through the steam box.

4. The system of claim 3 wherein the steam box is configured for a temperature of between about 175 degrees Fahrenheit and 210 degrees Fahrenheit and a relative humidity of between about 60 percent and 90 percent.

5. The system of claim 3 wherein the plurality of rollers define a fabric path of at least 8 linear yards.

6. The system of claim 5 wherein the plurality of rollers are configured to rotate at a speed sufficient to expose the spray dyed fabric to steam for at least 3 minutes.

10 7. The system of claim 1 wherein the first rinse station comprises:

- (a) a first pair of rinse spray nozzles, one of the pair directed to spray a rinse fluid downwardly onto incoming dyed fabric, and the other of the pair directed to spray a rinse fluid upwardly onto the incoming dyed fabric; and
- (b) a pair of nip rollers downstream for the first pair of rinse spray nozzles for extracting the rinse fluid.

15 8. The system of claim 7 wherein one of the pair of rinse spray nozzles is directed vertically downward onto the incoming dyed fabric, and the other of the pair directed vertically upward onto the incoming dyed fabric.

20 9. The system of claim 8 further comprising a second pair of rinse spray nozzles downstream of the first pair of rinse spray nozzles and upstream of the nip rollers, one of the second pair directed angularly downward onto the dyed fabric toward the nip rollers and the other of the pair directed angularly upward onto the dyed fabric toward the nip rollers.

25 10. The system of claim 1 further comprising a second rinse station downstream of the first rinse station, wherein the second rinse station comprises:

- (a) a pair of rinse spray nozzles;
- (b) a pair of nip rollers downstream of the rinse spray nozzles; and
- (c) wherein one of the pair of rinse spray nozzles is directed angularly downward onto the dyed fabric toward the nip rollers and the other of the pair is directed angularly upward onto the dyed fabric toward the nip rollers.

30 11. The system of claim 1 further comprising a dryer downstream of the at least one rinse station.

12. A process for dyeing tubular knitted fabric, comprising:

- (a) continuously moving the fabric in a machine direction;
- (b) opening the fabric with a spreader bar or former to flatten the fabric, wherein the fabric has a first outer surface above the spreader and a second outer surface below the spreader, and a width;
- (c) drawing the fabric over a roller having a plurality of raised ribs for maintaining tension in the fabric;
- (d) advancing the fabric through a dye station and spraying the first and second outer surfaces of the flattened fabric with a dye evenly across the width of the fabric; and
- (e) advancing the fabric through a fixation station and exposing the fabric to atmospheric steam to chemically react and affix the dye to the fabric.

15 13. The process of claim 12 wherein the dye spray saturates the fabric to between about 65 percent and 85 percent.

14. The process of claim 12 wherein the atmospheric steam is between about 175 degrees Fahrenheit and 210 degrees Fahrenheit and between about 60 percent relative humidity and 90 percent relative humidity.

20 15. The process of claim 14 wherein the fabric is exposed to the atmospheric steam for at least 3 minutes.

16. The process of claim 12 further comprising applying heat to the fabric to act as a catalyst to start the reaction of the dye with the fabric before advancing the fabric through the fixation station.

25 17. The process of claim 12, further comprising advancing the dyed fabric through at least one rinse station and rinsing off unfixed dye from the dyed fabric, using a plurality of spray nozzles, after exposing the fabric to the atmospheric steam.

30 18. The system of claim 1, wherein the roller having a plurality of raised ribs comprises a scroll roll having angled ribs diverging outwardly from a center of the roller toward opposed ends of the roller, the angled ribs formed to pull the fabric outwardly toward the opposed ends when the scroll roll rotates.

35 19. The process of claim 12, wherein the raised ribs of the roller are angled to pull the fabric outwardly toward opposed ends of the roller when the roller rotates.

\* \* \* \* \*